

Jan. 5, 1954

H. J. EDING ET AL  
ANALYSIS OF NONFERROUS ALLOYS

2,665,412

Filed March 31, 1952

3 Sheets-Sheet 1



FIG. 1

INVENTORS  
HAROLD J. EDING  
CLARENCE I. GLASSBROOK  
BY *Kenneth Swartwood*

ATTORNEY

Jan. 5, 1954

H. J. EDING ET AL

2,665,412

ANALYSIS OF NONFERROUS ALLOYS

Filed March 31, 1952

3 Sheets-Sheet 2



FIG. 2

INVENTORS

HAROLD J. EDING  
CLARENCE I. GLASSBROOK  
BY *Kenneth Swanson*  
ATTORNEY

Jan. 5, 1954

H. J. EDING ET AL

2,665,412

ANALYSIS OF NONFERROUS ALLOYS

Filed March 31, 1952

3 Sheets-Sheet 3



FIG. 3

INVENTORS  
HAROLD J. EDING  
CLARENCE I. GLASSBROOK  
BY *Kenneth Swartwood*  
ATTORNEY

## UNITED STATES PATENT OFFICE

2,665,412

## ANALYSIS OF NONFERROUS ALLOYS

Harold J. Eding, Palo Alto, and Clarence I. Glassbrook, Hayward, Calif., assignors to Ethyl Corporation, New York, N. Y., a corporation of Delaware

Application March 31, 1952, Serial No. 279,662

8 Claims. (CL 324—71)

1

This invention relates to the analysis of non-ferrous alloys. More particularly, the invention relates to a new and improved method for rapid or practically instantaneous analysis of molten non-ferrous alloys and to novel apparatus therefor.

The preparation of alloys for many purposes is frequently a time-consuming operation. This is particularly the case when a precise composition of alloy is essential, as for example in producing metallic alloy compounds for chemical purposes. Foremost among such instances are the alloys of lead, particularly with the alkali metals or the alkaline earth metals. Such alloys include, for example, sodium-lead alloys, magnesium-lead alloys, calcium-lead alloys, ternary alloys containing lead, sodium and potassium, and potassium-lead alloys, and the like. Foremost among alloys of this nature is the monosodium alloy of lead, NaPb, containing 10 weight percent sodium and 90 percent lead. This monosodium alloy is widely used in the manufacture of the alkyllead compounds, particularly tetraethyllead.

The prior commercial methods employed for the preparation of the lead-sodium alloys may be considered typical of the time-consuming procedures necessary. Thus, in the manufacture of an alloy containing 10 weight percent sodium, the ordinary procedure has been to mix molten lead and molten sodium to the approximate composition required, using the weights of materials as guides. Upon the completion of the mixing operation, it has been customary to take a sample and carry out the chemical analysis to determine what corrective action must be taken to arrive at the final precise composition necessary. The method of analysis heretofore used has been to contact the alloy sample with mercury and a standard amount of acid of known concentration. After complete reaction of the sodium content of the alloy, the residual or excess acid is back-titrated with a caustic solution to determine the amount of sodium metal present. This method, while accurate, involves the usual delay of chemical analytical procedures, and has caused the hold-up of production while such laboratory analysis was carried out. Obviously, the time required for such analysis to determine what corrective action was required is a bottle-neck in the manufacturing operations. A more rapid and precise analytical technique was therefore desired.

The object of the present invention is to provide a method and apparatus for the analysis of molten metal alloys without the necessity of chemical

2

manipulation. A further object is to provide apparatus which is relatively simple and requires no special skill in operation thereof. A further object is to provide a method and apparatus therefor capable of a high degree of reproducibility and accuracy in a long series of repetitive determinations. Other objects will appear hereafter.

It has now been discovered that the composition of a molten alloy can be ascertained with a great degree of precision by determining the electrical potential difference or voltage difference between the alloy and a reference metal of known composition. The reference metal as well as the alloy should be in the molten state and preferably at the same temperature. A specimen of the reference metal is maintained adjacent to the alloy being analyzed, and is contained within a capsule of non-metallic material, the capsule being of thin glass or some other vitreous composition. Broadly, therefore, the method of the invention comprises placing a specimen of the molten reference metal within a body of the alloy being analyzed, but separated from admixture therewith by a barrier or liquid tight capsule container which is permeable at operating temperatures to ions of the metal being determined. The reference metal specimens so placed is, however, electrically isolated from the surface of the alloy body. The voltage developed between the alloy proper and the reference metal specimen is measured and is a function of and an indication of the composition of the alloy.

The reference metal can be any of a number of different compositions. In most instances, a pure specimen of the metal being determined in the alloy will be used, but an alloy or mixture of such a metal with a different metal is frequently used. In other instances, an equivalent metal will be used, that is, the reference metal will not include or consist of the metal being determined by the analysis.

It has been found essential that a truly representative voltage difference be ascertained between the alloy being analyzed and the reference metal. By this is meant that certain obscuring voltages, having no relation to the voltage difference between the alloy proper and the reference metal, are screened out or prevented from being impressed on the voltage between the alloy proper and the reference metal. It has been found that if this is not done, that not only is the representative voltage not ascertainable at the start, but on continued usage of a particular apparatus,

the obscuring voltages increase with time so there is no opportunity for standardization.

The above mentioned obscuring voltages are apparently resultant from impurities or contaminants on the surface of the alloy being analyzed when in contact with the apparatus used. In order to negate the adverse effect of such obscuring voltages, it is essential to provide electrical isolation of the reference metal specimen from the surface of the alloy.

The method of the invention and the best manner of use will appear from the detailed description given hereafter and from the figures. Figure 1 illustrates typical requisite apparatus for carrying out the method, including a voltage measuring instrument, electrical conductors for transmitting the voltage of the alloy and of the reference metal, and a reference metal assembly. Figure 2 shows a typical relationship between the composition of an alloy, of sodium and lead, and a voltage developed between such an alloy and reference metal consisting of sodium. Figure 3 is a schematic illustration of auxiliary electrical apparatus receiving and indicating the voltage difference signal measured between the alloy and the reference metal and for providing a further refinement in accuracy.

Referring to Figure 1, the essential elements of apparatus for employing the method are shown, these including a reference metal assembly 11, an alloy potential wire 12 for ascertaining the electrical potential of the alloy being analyzed, and a voltage measuring instrument 13. The reference metal holder 11 is partially immersed in the alloy 22, and the alloy wire 12 has its terminus, which may be a small coil 24, also immersed in the alloy sample. A voltage difference between a reference metal specimen 18 and the alloy 22 is transmitted by wires 12, 17 to the voltmeter 13 for measurement and indication.

The reference metal holder 11 includes a capsule 14 in the form of an elongated tube of circular cross section, a sleeve 15, a protective sheath 16 and an electrical lead wire 17. The lead wire 17 enters the capsule 14 through a gas tight seal 27 and is normally positioned concentrically in the capsule. The terminus of the wire 17, usually a short coil 26, is immersed in the reference metal specimen 18.

The capsule 14 and the sleeve 15 are made of the same material, e. g., a heat resistant glass, the sleeve being permanently joined to the capsule wall in preparation. The annular space 20 between the capsule and sleeve is open to the atmosphere. In some instances the sleeve may be joined to the capsule at top and bottom. The protective sheath 16 is of a metal resistant to corrosive attack by the alloy being analyzed, iron or steel being suitable for most purposes. The protective sheath may be in a number of mechanical forms, a preferred shape being a shouldered cylindrical bushing as shown. The sheath 16 fits fairly snugly about the sleeve 15, and has a shoulder 31 at the topmost extremity which rests on the wall 30 of the alloy conduit or vessel. Usually a packing 32 is wedged in between the bottom of the sheath 16 and the sleeve 15 to provide a liquid and gas tight seal. The packing or seal material may be of asbestos fibers, or asbestos plus sauerisen cement or a similar sealing material which is inert to the alloy at the temperatures involved. In addition to providing a fluid seal, the packing material 32 provides for mechanical support of sleeve and capsule in operation.

In virtually all instances it is highly desirable that the free space 19 within the capsule 14 (not occupied by the reference metal specimen 18) should be filled with an inert gas. Suitable gases are argon, helium, nitrogen or an alkane hydrocarbon gas. The exclusion of any gaseous component which could react with the reference metal precludes the possibility of reaction products creating an obscuring voltage by contact

10 with the lead wire 17. In constructing and filling the capsule 14 of the reference metal holder, the lead wire is usually first inserted and a gas tight seal 27 is formed. A short branch or nipple is part of the unfilled capsule and serves as the filling port for the reference metal and for the inert gas protective blanket. After charging the capsule this nipple is closed, preferably by fusion of the glass, leaving a slight projection 25 as shown.

In this form of reference metal assembly, it is essential that the seal or point of entry 27 of the lead wire 17 into the capsule be gas tight. This may be accomplished in several ways. For example, a metal having an expansion coefficient 20 near to that of glass, such as tungsten, may be used. In such cases, the portion of the wire 17 passing through the capsule wall is made of such a metal and is sealed in a conventional manner, by melting and pinching the glass nipple about 25 the wire. An alternative and preferred mode of 30 making this seal involves melting a supply of silver chloride about the junction of the lead wire and the capsule wall, which has been found to provide a highly efficient seal.

35 A closed and sealed reference metal capsule as shown is the preferred mode of protecting the purity of the reference metal. However, the same degree of protection can be realized even if the capsule container is open at the top end. 40 For such embodiments, a continuous small stream of a pure, dry inert gas is passed into the capsule. This method of operation of course requires more frequent attention than necessary when a sealed capsule is employed, but nevertheless provides reproducible, accurate results.

45 In operation, the reference metal holder is partially immersed in a sample or stream of molten alloy 22. The protective sheath 16 projects through the surface of the alloy. It has been found that alloy melts are apparently covered by a thin, almost imperceptible film 21 of products of corrosion of the alloy, or slag impurities, which tend to attack the material of the sleeve 15. The sheath thus prevents such contact and corrosion.

50 55 It will be noted that the surface 29 of the specimen 18 of the reference metal occupies an elevation, when the assembly is in operation, which is somewhat below the seal of the sleeve 15 with the capsule 14. This disposition of the reference metal specimen is not particularly significant with respect to the operability of the method, but is desirable in minimizing thermal strains at the seal 28.

60 65 In contrast to the reference metal elevation, the disposition of the seal point 28 with respect to the sheath 16 is of great importance in the apparatus. It has been found that adequate distance between these two points is essential for 70 providing the necessary electrical isolation. This separation distance is not precisely ascertainable in advance for all installations, as the magnitude of obscuring voltages, apparently associated with the surface of an alloy sample, are variable according to the concentration and identity of the

components of the alloy. In general, however, it is found that providing a separation distance—that is, the linear distance between the sheath 16 lower extremity and the seal 28—at least ten times the wall thickness of the capsule, will provide a high degree of isolation. As the capsule will ordinarily be made of material having a wall thickness of less than 1 millimeter, a separation distance of the order of about one-half to one inch provides an ample margin of safety. In those instances wherein a metal sheath is not used, the separation distance requirement refers to the distance from the alloy surface to the joint of the sleeve with the capsule.

Surprisingly, the desired electrical isolation cannot be achieved by merely extending the length of the capsule 14 or by other more or less obvious measures. For example, it would be theorized that if capsule 14 were sufficiently long in dimension, and the wire 17 did not touch the interior walls other than at the point of seal 27, that merely by having the reference metal specimen sufficiently far below the level 21 of the alloy sample, that electrical isolation would be achieved. However, numerous tests have shown that this is not the case, and that an inaccurate and variable voltage is measured. It is believed that at the high temperatures of operation, a thin film of reference metal is vaporized and deposited on the interior walls of the capsule. This thin film, even though of extremely thin proportions, is sufficient to transmit obscuring voltages to the reference metal specimen proper or directly to the wire 17. A sleeve 15, such as is illustrated, joined to the capsule at 35 a point 28 removed from the sheath 16 by the above-mentioned separation distance is thus essential to the method.

As the above described combination provides electrical isolation of the entire capsule, it is 40 immaterial whether the wire 17 touches the interior walls of the capsule. This makes possible particularly compact assemblies when desired. Thus, the capsule may have a restricted diameter portion, say about one-fourth inch, above a bulb portion holding the reference metal specimen. As heretofore mentioned, the wire 17 may be in 45 contact with the walls so that concentricity is not essential. In addition the reference metal specimen may be of such volume that it occupies a portion of the restricted diameter section of the capsule. No particular benefit is realized from such an increase in volume of the reference metal specimen, however, and in all instances wherein a sealed capsule is used a certain amount of free space is necessarily provided. Such free space is needed to prevent stresses and cracking of the capsule owing to expansion of the metal specimen with temperature changes.

The two lead wires 12, 17 are made of the same 60 metal, pure soft iron thermocouple wire being a preferred material. The terminus 24 of the wire 12 to the alloy sample is located quite near to the reference metal holder, and at about the same immersion, so that the temperatures at these two points will be the same.

An alternative but generally less satisfactory mode of obtaining the voltage of the alloy proper is to connect the conductor 12 to the metal container or conduit for the alloy at a point adjacent to the reference metal specimen holder. This 70 procedure is less satisfactory because of the likelihood of errors being introduced because of voltages being generated through differences in composition of the metal container for the alloy and 75

of the conductor 17 for ascertaining the potential of the reference metal specimen.

The chart of Figure 2 illustrates a typical voltage-composition relationship such as is utilized by the present method. Referring to Figure 2, these relationships are given for an alloy comprising sodium and lead, curve A being for a uniform temperature of 440° C. and curve B being for a temperature of 450° C. It will be seen that ascertaining the voltage difference between a sodium-lead alloy and pure sodium metal affords a rapid and precise method for determining its composition. Thus, at 440° C., for example, a millivoltage of 197 shows that the alloy contains 10 weight percent sodium, while an increase in voltage to 200 mv. indicates that the alloy contains 9.88 percent sodium. The curves of Figure 2 were prepared by determining the voltage difference exhibited between a series of alloys of known composition and pure sodium. For other systems, similar operational data are readily determined.

As previously indicated, the usual shape of the reference metal capsule is an elongated tube having a hemispherical bottom. The shape and size of the reference metal specimen has been found to be of little importance with respect to accuracy of the method. An examination of performance of different shapes of capsules has shown no evidence of a potential of asymmetry. In all cases, for practical reasons of assembly, it will be desirable to provide a capsule of about one-half inch internal diameter at the locus of the reference metal specimen.

With reference to the vitreous material utilized for the capsule and the sleeve of the reference metal holder, a heat and shock resistant glass is preferred. The precise mode of operation of the vitreous material with respect to establishing the measurable voltage difference is not completely understood. It has been found that such materials are dielectrics, that is, electron flow is not obtained through the walls. Nevertheless, at the temperatures of the molten alloy being analyzed, these materials are permeable in varying degrees to the positive ions of light metals such as sodium, potassium, lithium or the alkaline earth metals. The analysis of a very satisfactory glass of this type is as follows, compositions in weight percent: 80.5 SiO<sub>2</sub>, 2.2 Al<sub>2</sub>O<sub>3</sub>, 3.8 Na<sub>2</sub>O, 0.4 K<sub>2</sub>O and 12.9 BeO<sub>3</sub>. Other glasses have been used with very satisfactory results. However, not all glasses have adequate resistance to thermal shock. For example, although a capsule 55 made of a glass containing about 19 percent sodium oxide has proven very acceptable with respect to analysis of a sodium-lead alloy, it is fairly rapidly attacked owing apparently to its low physical strength at the elevated temperatures of operation. Consequently, its effective service life is limited. As a general rule, the capsule material should include as a component the oxide of the metal being determined in the alloy, although such oxide may be present in low concentrations. As an alternative to the construction here illustrated, the capsule and the sleeve walls may be strengthened by circumferential wire bands within the wall. Ordinarily, however, such elaboration is not necessary.

Generally, the wall thickness of the capsule does not affect the potential accuracy of determination of the voltage difference to be ascertained. The wall thickness does, however, affect the ease with which the voltage difference is measured. This arises because an increase in

the capsule wall thickness increases the electrical resistance of the system and requires further refinements in the external electrical circuit. For these reasons, a capsule wall thickness of about one-half to one millimeter is preferred.

Each of the several components of the reference metal holder are important for obtaining the full benefits of the invention. The protective metal sheath 16 may be dispensed with when desired, its function being to provide chemical and mechanical protection of the capsule and sleeve. In addition, the protective sheath provides a mounting or support whereby the assembly is positioned within a conduit, pipe or vessel holding the alloy.

Although the protective metal sheath may be eliminated, the integral combination of the capsule and the sleeve is highly desirable in all practical forms of the apparatus to provide the isolation of the reference metal specimen. The importance of this combination is illustrated by the following examples.

#### Example I

A reference metal holder resembling the holder illustrated by Figure 1 was prepared, except that no sleeve was used. The assembly was charged with pure metallic sodium and sealed. The assembly was inserted in a molten sample of sodium-lead alloy containing 9.68 weight percent sodium, maintained at about 440° C. The millivoltage difference between the reference sodium and the alloy sample was measured in a conventional manner and recorded for a period of about two weeks of steady operation. It was found that the voltage difference measurement failed to remain constant, but steadily increased with time. Thus, the initial voltage was 212 mv., and after 5, 10, and 12 days' operation the voltage measured was 430, 570, and 1168 mv., respectively. It is apparent that the reference metal holder of this test would be entirely unsatisfactory for analyzing an alloy sample.

#### Example II

A reference metal holder such as is described heretofore, and as illustrated by Figure 1, was made of boro-silicate glass and charged with pure sodium metal. As in the previous example, the reference voltage wire made occasional contact with the capsule walls above the level of the alloy specimen. The instrument was used for measuring the voltage difference between the sodium specimen and sodium-lead alloy having 9.68 weight percent sodium and maintained at about 440° C. Measurements were taken continuously over a period approaching four weeks. The voltage readings varied less than one-half percent during this period.

The foregoing examples illustrate the importance of providing electrical isolation of the reference metal specimen from the alloy sample surface and the efficacy of our apparatus in this regard. It has been found that the method of analyzing an alloy is extremely versatile. For example, it is not essential that the reference metal be identical with the component being determined in the alloy. As an example of such usage, sodium can be employed as the reference metal in determining the amount of potassium in a ternary alloy of sodium, potassium and lead. In such instances, it will be necessary to ascertain the amount of sodium present, by application of the method to the binary alloy of sodium and lead, before addition of the potassium component.

The addition of potassium to the alloy produces the same effect on the voltage difference as the addition of a stoichiometric equivalent of sodium metal. It will therefore be apparent that the procedure is applicable to the analysis of multi-component alloy systems.

In general, it is possible to prepare or manufacture completed reference metal assemblies which are interchangeable. As a practical matter, it is highly desirable to make at least one calibration determination before using a new assembly. The necessity of such a check run arises because of the possibility of inclusion of small amounts of impurities in the reference metal specimen which would have the effect of altering the voltage readings slightly.

The instrument for measuring the voltage difference may be of several different types. Thus, a manually operated potentiometer may be used. A conventional voltmeter is, however, not suitable, inasmuch as the high internal resistance of the capsule wall will introduce an error in the voltmeter reading. In order to obtain the maximum accuracy, it will frequently be desirable to employ a "bucking" voltage, so that a voltage measuring instrument of greater sensitivity can be used. Figure 3 illustrates schematically an electrical circuit for such cases.

Referring to Figure 3, elements are shown of an embodiment for attaining a record of composition with a high degree of precision. Such elements include of course the reference metal assembly inserted in place in a body of the alloy and appropriate electrical leads for transmitting the voltage developed. In addition electrical apparatus is supplied for applying a suppressing or "bucking" voltage, opposite in direction to the voltage developed, and appropriate indicating recording apparatus.

The suppression voltage has been found to contribute to the accuracy of the record of analysis obtained in the following manner. In a particular operation, ordinarily, the alloy components can be easily blended in approximately the desired proportions. Therefore, the analyses will usually be of alloys deviating only minor amounts from the desired final precise composition. Accordingly, it will then not be necessary to measure voltages over the entire scope of voltages developed by the reference metal-alloy combination. Therefore, by applying a constant bucking voltage corresponding to the voltage developed when the alloy is at or near the desired composition, the residual voltage (difference between the actual developed and the "bucking" voltages) can be measured most accurately by employing an instrument providing the highest sensitivity for the small variation in residual voltage.

As an illustrative example, considering the manufacture of monosodium-lead alloy, a voltage of the order of 195 millivolts is approximately the voltage developed by this alloy at its desired composition. By applying a suppressing voltage of slightly less than 195 millivolts and measuring the residual voltage with an instrument capable of measuring over a span of only five millivolts with an accuracy of about one percent, a net accuracy in voltage measurement of 0.005 percent, with corresponding precision in determining alloy composition, is readily attained.

It will be readily apparent that, in order to obtain the benefits of a suppression voltage, it must be applied with a high degree of precision and stability. The embodiment of Figure 3 illustrates circuiting providing such precision.

Referring to Figure 3, the electrical lead 43 from a reference metal specimen assembly 42 is connected to a resistor 45. Also joined at this point is a lead wire 46 from a conventional dry cell 47 (or other semi-permanent direct current source) in opposite polarity to the voltage developed. A standard cell 48 is connected across a fixed resistor 49 in opposite polarity to the dry cell 47. The standard cell 48 is connected to the resistor 49 through an amplifier 50.

A third resistor 51 of variable capacity is adjusted by a balancing motor 52 in response to impulses from the amplifier 50. The resistor 49 is so chosen that when sufficient current flows in the battery circuit to create a voltage drop in resistor 45 exactly equal to the desired suppression voltage, then the concurrent voltage drop in resistor 49 is equal to the voltage of the standard cell 48. Any unbalance with respect to the cell 48 and resistor 49 is detected by amplifier 50 which transmits a power impulse to balancing motor 52 which adjusts variable resistor 51 to provide the desired voltages across resistors 49 and 45.

It has been found that the above described circuiting is capable of extremely high precision in providing a suppression voltage. A stability of better than one part in 10,000 has been obtained in providing a suppression voltage of 192.5 millivolts.

The discharge wire 53 from the voltage suppression section and the wire 44 from the alloy sample therefore provide a residual voltage to a recorder 54, the said residual voltage being practically instantaneously responsive to the composition of the alloy. The recorder 54 may be any of a number of readily available instruments and is fitted with proper adjustments to provide maximum sensitivity over the voltage range to be applied thereto.

Having described our process and apparatus and the preferred embodiments thereof, what we desire to claim is:

1. The process for analyzing a molten non-ferrous alloy comprising immersing a liquid reference metal specimen in a body of the alloy but separated therefrom by a barrier of a vitreous material permeable to ions of the metal being determined, electrically isolating the reference metal specimen from the surface of the alloy, establishing an electrical connection between the alloy and the said reference metal specimen and measuring the voltage developed between the alloy and the reference metal.

2. The process for analyzing a molten alloy of lead with at least one alloying metal selected from the group consisting of alkali and alkaline earth metals, comprising immersing a molten reference metal specimen in a body of the alloy but separated therefrom by a barrier of a vitreous material permeable to ions of the metal being determined, electrically isolating the reference metal from the surface of the alloy, establishing an electrical connection between the alloy and the said reference metal specimen and measuring the voltage developed between the alloy and the reference metal.

3. The process of claim 2 further defined in that the alloy consists essentially of lead and sodium and the reference metal consists essentially of sodium.

4. The process of claim 2 further defined in that the alloy consists essentially of lead, sodium, and potassium, and the reference metal consists essentially of sodium.

5. The process for analyzing a molten alloy of lead and sodium comprising immersing a molten specimen of sodium in a body of the alloy but separated therefrom by a barrier of borosilicate glass, electrically isolating the specimen of sodium from the surface of the alloy, establishing an electrical connection between the alloy and the sodium specimen to transmit the voltage developed between the alloy and the sodium, applying a constant suppression voltage to said developed voltage, and measuring the difference in voltage between the developed and suppression voltages.

6. A reference metal assembly for placing a specimen of reference metal within a body of molten alloy but electrically isolated from the surface of the alloy comprising a capsule adapted for partial immersion in the alloy; a surrounding sleeve defining an annular space therewith and circumferentially sealed to the capsule to prevent entry of the alloy to the annular space; a molten reference metal specimen within said capsule; and an electrical conductor into the capsule and in electrical contact with the reference metal specimen; said conductor being electrically isolated from the molten alloy, and the capsule and the sleeve being of a dielectric vitreous material permeable to ions of a metal component of the alloy.

7. A reference metal assembly for placing a specimen of reference metal within a body of molten alloy but electrically isolated from the surface of the alloy comprising an elongated closed capsule adapted for partial immersion in the alloy; a surrounding sleeve defining an annular space therewith and circumferentially sealed to the capsule to prevent entry of the alloy to the annular space; a molten reference metal specimen within said capsule; and an electrical conductor extending through a wall portion of the capsule and in electrical contact with the reference metal specimen, said wall portion being remote from the reference metal specimen and electrically isolated from the molten alloy, and the capsule and sleeve being of a dielectric vitreous material permeable to ions of a metal component of the alloy.

8. A reference metal assembly for placing a specimen of molten sodium metal within a body of molten sodium-lead alloy but in electrical isolation from the surface of the alloy, comprising an elongated, closed capsule adapted for partial immersion in the alloy; a surrounding sleeve defining an annular space therewith and circumferentially sealed to the capsule to prevent entry of the alloy to the annular space; a molten specimen of sodium within said capsule; and an electrical conductor extending through a wall portion of the capsule and in electrical contact with the molten sodium specimen; said wall portion being remote from the molten sodium specimen and electrically isolated from the molten alloy, and the capsule and sleeve being of borosilicate glass.

HAROLD J. EDING.  
CLARENCE I. GLASSBROOK.

References Cited in the file of this patent

UNITED STATES PATENTS

| Number    | Name    | Date          |
|-----------|---------|---------------|
| 2,342,029 | Zubko   | Feb. 15, 1944 |
| 2,366,844 | Doschek | Jan. 9, 1945  |